# EUROPEAN PATENT SPECIFICATION

(11) **EP 2 835 417 B1**
(45) Date of publication and mention of the grant of the patent: **17.10.2018**
(21) Application number: 13769463.4
(22) Date of filing: 01.04.2013
(51) Int. Cl.: C10M 171/00, C10G 45/46, C10G 45/64, C10G 47/12, C10G 65/08, C10G 65/12, C10M 101/02, C10M 105/04, C10M 177/00, C10N 20/00, C10N 20/02, C10N 30/00, C10N 30/02, C10N 40/00, C10N 40/02, C10N 40/04, C10N 40/06, C10N 40/08, C10N 40/12, C10N 40/16

(54) **LUBRICANT BASE OIL**
SCHMIERMITTELBASISÖL
HUILE DE BASE POUR LUBRIFIANT

(30) Priority: 30.03.2012 JP 2012082349; 30.03.2012 JP 2012082354; 30.03.2012 JP 2012082393; 30.03.2012 JP 2012082406; 30.03.2012 JP 2012082446; 30.03.2012 JP 2012082457
(43) Date of publication of application: 11.02.2015
(73) Proprietor: JX Nippon Oil & Energy Corporation, Chiyoda-ku Tokyo 100-8162 (JP)
(72) Inventor: TAGAWA Kazuo, Tokyo 100-8162 (JP); HAYASAKA Kazuaki, Tokyo 100-8162 (JP)
(74) Representative: Grünecker Patent- und Rechtsanwälte PartG mbB
(86) International application number: PCT/JP2013/059947
(87) International publication number: WO 2013/147302

(56) References cited:
- JP-A- 2006 509 899
- JP-A- 2006 518 395
- JP-A- 2006 521 416
- JP-A- 2007 516 337
- JP-A- 2011 506 677
- US-A1- 2005 261 146
- US-A1- 2007 238 628
- US-A1- 2011 237 477

## Description

### Technical Field

The present invention relates to a lubricant base oil.

### Background Art

Conventionally, regarding a lubricant base oil and a lubricant oil composition, satisfaction of both a high viscosity index and a low-temperature viscosity characteristic has been attempted.

For example, by blending an additive agent such as a pour-point depressant into a lubricant base oil such as a highly-refined mineral oil, improvement of a low-temperature viscosity characteristic of a lubricant oil has been attempted (for example, refer to Patent Literature 1 to 3). Moreover, as a producing method of a high viscosity index base oil, for feedstock containing natural and synthetic normal paraffins, a method of refining a lubricant base oil by hydrocracking/hydroisomerization is known (for example, refer to Patent Literature 4 to 6).

A pour point is generally as an evaluation index of a low-temperature viscosity characteristic of a lubricant base oil and a lubricant oil. In addition, a technique for evaluating a low-temperature viscosity characteristic based on a lubricant base oil such as the content of normal paraffins and isoparaffins is also known.

### Citation List

### Patent Literature

Patent Literature 1: JP-A-04-036391
Patent Literature 2: JP-A-04-068082
Patent Literature 3: JP-A-04-120193
Patent Literature 4: JP-A-2005-154760
Patent Literature 5: JP-T-2006-502298
Patent Literature 6: JP-T-2002-503754

US 2011/237477 A1 relates to a hydrocarbon-based lubricating base oil, wherein a urea adduct value is not greater than 4% by mass, a viscosity index is 100 or higher, an average of carbon atoms number is 23 to 31 as determined by gas chromatography distillation, a value obtained by dividing an integral value of a peak in 30 ppm by an integral value of total peaks in the range of from 0 ppm to 50 ppm for the ¹³C-NMR spectrum is 0.1 to 0.2, and a product of a value obtained by dividing an integral value of peaks attributed to tertiary carbon atoms by an integral value of total peaks in the range of from 0 to 50 ppm for the ^{l3}C-NMR spectrum, and the average of carbon atom numbers is 1.8 to 2.5.

US2007/238628 A1 relates to a multigrade automotive gear lubricant, comprising:
- between 5 and 95 wt % of a base oil, made from a waxy feed, having a traction coefficient less than 0.021 when measured at a kinematic viscosity of 15 cSt and at a slide to roll ratio of 40 percent;
- less than 2 weight percent viscosity index improver or other thickener; and
- an EP gear lubricant additive.

US 2005/261146 A1 discloses a process for producing a lubricant blend comprising:
a) providing a lubricant oil fraction derived from highly paraffinic wax having a viscosity of between 2 cSt and 20 cSt at 100°C, wherein the lubricant oil fraction derived from highly paraffinic wax comprises:
   - less than 0.30 weight percent aromatics
   - greater than 5 weight percent molecules with cycloparaffinic functionality; and
   - a ratio of weight percent of molecules with monocycloparaffinic functionality to weight percent of molecules with multicycloparaffinic functionality greater than 15;
b) blending the lubricant oil fraction derived from highly paraffinic wax with a petroleum derived base oil selected from the group consisting of a Group II base oil, a Group III base oil, and mixtures thereof; and a pour point depressant; and
c) isolating a lubricant blend having a Brookfield viscosity at -40°C of less than 100,000 cP.

### Summary of Invention

### Technical Problem

As described above, in general, it is considered that lower cold flow property of a lubricant base oil is better, and according to the study of the present inventors, a conventional lubricant base oil having cold flow property has a problem in a sealing property. More specifically, a low viscosity of a lubricant base oil or, moreover, contraction of a sealing material widens a gap, and when a pressure is applied to the site, oil leakage becomes easy to occur.

The present invention has been made in view of these circumstances, and it is an object of the present invention to provide a lubricant base oil capable of satisfying both a low-temperature viscosity characteristic and a sealing property at a high level.

### Solution to Problem

In order to achieve the above-described object, firstly, the present inventors attempted satisfaction of both a low-temperature viscosity characteristic and a sealing property of a lubricant base oil using an SBV viscosity as an index, as an approach different from improvement in a low-temperature viscosity characteristic of a lubricant base oil using a pour point as an index. As a result, it was found that when the kinematic viscosity at 100°C, viscosity index, and SBV viscosity at -20°C of a lubricant base oil satisfy their respective specific requirements, a sealing property can be improved while sufficiently maintaining a low-temperature viscosity characteristic to complete the present invention.

That is, the present invention provides in embodiments:
a lubricant base oil that is a hydrocarbon oil that satisfies any of the following conditions (i), (ii) and (iii):
   (i) a hydrocarbon oil having a kinematic viscosity at 100°C of 3.0 to 5.0 mm²/s, a viscosity index of 145 or more, and an SBV viscosity at-20°C of 3,000 to 60,000 mPa·s, the viscosity being determined in accordance with ASTM D5133,
      wherein the hydrocarbon oil has a ratio of CH₂ carbons constituting a main chain to all carbons constituting the lubricant base oil of 15% or more in a ¹³C-NMR analysis, wherein ¹³C-NMR analysis is performed under the following conditions:
      a diluted sample obtained by adding 3 g of deuterated chloroform to 0.5 g of a sample is used, the measurement temperature is room temperature, the resonant frequency is 100 MHz, and a gated decoupling method is used,
      wherein the hydrocarbon oil has a cycloparaffin content of 50% or less in an FD-MS analysis, wherein the FD-MS analysis is performed under the following analysis conditions:
         a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min,
   (ii) a hydrocarbon oil having a kinematic viscosity at 100°C of 5 to 9 mm²/s, a viscosity index of 155 or more, and an SBV viscosity at-20°C of 3,000 to 30,000 mPa·s,
      wherein the hydrocarbon oil has a ratio of CH₂ carbons constituting a main chain to all carbons constituting the lubricant base oil of 20% or more in a ¹³C-NMR analysis, wherein ¹³C-NMR analysis is performed under the following conditions:
      a diluted sample obtained by adding 3 g of deuterated chloroform to 0.5 g of a sample is used, the measurement temperature is room temperature, the resonant frequency is 100 MHz, and a gated decoupling method is used,
      wherein the hydrocarbon oil has a cycloparaffin content of 60% or less in an FD-MS analysis, wherein the FD-MS analysis is performed under the following analysis conditions:
      a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min, and
   (iii) a hydrocarbon oil having a kinematic viscosity at 100°C of 2.0 to 3.0 mm²/s, a viscosity index of 130 or more, a pour point of -27.5°C or more, and an SBV viscosity at -30°C of 1,000 to 30,000 mPa·s
      wherein the hydrocarbon oil has a ratio of CH₂ carbons constituting a main chain to all carbons constituting the lubricant base oil of 15% or more in a ¹³C-NMR analysis, wherein ¹³C-NMR analysis is performed under the following conditions:
      a diluted sample obtained by adding 3 g of deuterated chloroform to 0.5 g of a sample is used, the measurement temperature is room temperature, the resonant frequency is 100 MHz, and a gated decoupling method is used;
      wherein the hydrocarbon oil has a cycloparaffin content of 30% or less in an FD-MS analysis, wherein the FD-MS analysis is performed under the following analysis conditions:
         a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min,
         wherein the content of the saturated content in the lubricant base oil on the basis of the total amount of the lubricant base oil is 90% by mass or more; and
         wherein the aromatic content in the lubricant base oil on the basis of the total amount of the lubricant base oil is 5% by mass or less.

### Preferred embodiments are set forth in the subclaims.

Here, the kinematic viscosity and the viscosity index in the present invention mean a kinematic viscosity and a viscosity index measured in conformity with JIS K 2283-1993, respectively.

Moreover, the SBV viscosity in the present invention means a value measured by a method in which a viscosity is continuously measured by rotating a rotor at 0.3 rpm while cooling at a cooling rate of 1°C/hour, which is a test method defined in ASTM D5133.

Moreover, the freezing point in the present invention means a value measured according to the following procedure.

More specifically, a sample charged in a test tube is preheated to 46°C, and then, is cooled at 2.5°C/min, and a cooling rate is changed to 1°C/min at a temperature higher than an expected freezing point (measured once in advance) by 10°C to start the measurement. According to this method, a reproducible freezing point can be obtained compared to JIS. This freezing point is distinguished from a pour point measured by JIS K 2269-1987 (JIS method pour point). In addition, according to the study of the present inventors, the pour point defined in JIS is suitable for measuring a liquid having widely differing crystallization temperatures, such as a petroleum lubricant base oil that is a multicomponent mixture. However, in the case of the present invention, a single component of paraffin does not flow by the JIS measurement method for evaluating fluidity when being inclined, but is confirmed to flow by the application of exogenous force and does not exhibit actual fluidity. The cause is due to the composition and is also affected by a rate of temperature decrease of 2.5°C/min, and determination in a situation where crystallization does not proceed completely is considered to be the cause. Therefore, it is necessary to accelerate fluidity of base oil molecules and to obtain a freezing point close to a true value by slowing a descending rate of temperature.

Moreover, the ratio of CH₂ carbons constituting the main chain to all carbons constituting the lubricant base oil can be determined, for example, by performing a ¹³C-NMR analysis under the following analysis conditions.

More specifically, in the present invention, in the ¹³C-NMR measurement, a diluted sample obtained by adding 3 g of deuterated chloroform to 0.5 g of a sample was used, the measurement temperature was room temperature, and the resonant frequency was 100 MHz. In addition, a gated decoupling method was used as the measurement method.

The ratio of CH₂ to the total of the constituent carbons of the lubricant base oil of the present invention means a ratio of the total of integral intensity attributed to the CH₂ main chain with respect to the total of integral intensity of all carbons, which are measured by ¹³C-NMR, and other methods may be used as long as the equivalent result is obtained.

Furthermore, the ratio of the cycloparaffin content can be determined, for example, by performing an FD-MS analysis under the following analysis conditions.

The FD method is an ionization method in which a sample is coated on an emitter, a current is applied to the emitter to heat the coated sample, and a tunneling effect is used in a high electrical field on the emitter surface and in the vicinity of the whisker tip. In the present invention, the measurement was performed using JMS-AX505H by JEOL Ltd. under conditions of an accelerating voltage (cathode voltage) of 3.0 kV and an emitter current of 2 mA/min. Compound types in mass spectrometry are determined by specific ions to be formed, and they are generally classified by a z value. The z value is represented by a general formula CₙH_{2n+z} for all hydrocarbon species. Since the saturated phase is analyzed separately from the aromatic phase, contents of different cycloparaffins having the same stoichiometry can be measured. In addition, cycloparaffins include both of monocyclic cycloparaffins and bicyclic or more cycloparaffins.

### Advantageous Effects of Invention

According to the present invention, a lubricant base oil capable of satisfying both a low-temperature viscosity characteristic and a sealing property at a high level.

### Description of Embodiments

Preferred embodiments of the present invention will now be described in more detail.

### [First Embodiment: Lubricant Base Oil that is Hydrocarbon Oil that satisfies Condition (i)]

The lubricant base oil according to the first embodiment of the present invention is a lubricant base oil that is a hydrocarbon oil having a kinematic viscosity at 100°C of 3.0 to 5.0 mm²/s and an SBV viscosity at -20°C of 3,000 to 60,000 mPa·s.

In addition, conventionally, a pour point used as an index of a low-temperature viscosity characteristic of a lubricant base oil evaluates ease of flow, that is to say, a bulk viscosity. In contrast, the SBV viscosity in the present invention can evaluate not a bulk viscosity but mobility of a base oil at the molecular level. For example, a lubricant base oil does not flow at a temperature lower than a pour point, but can move at the molecular level due to distortion between molecules constituting the base oil to impart the SBV viscosity. The lubricant base oil according to the present embodiment is made based on the above-described present inventors' knowledge, and has an unexpected significant effect that, in a lubricant base oil having a kinematic viscosity at 100°C of 3.0 to 5.0 mm²/s and a viscosity index of 145 or more, by making the SBV viscosity at -20°C of the lubricant base oil be 3,000 to 60,000 mPa·s, a sealing property can be improved while sufficiently maintaining a low-temperature viscosity characteristic.

The kinematic viscosity of the lubricant base oil according to the present embodiment at 100°C is 3.0 to 5.0 mm²/s, preferably 3.0 to 4.5 mm²/s, more preferably 3.2 to 4.3 mm²/s, and more preferably 3.4 to 4.1 mm²/s.

Moreover, the viscosity index of the lubricant base oil according to the present embodiment is 145 or more, preferably 147 or more, and more preferably 148 to 160. In addition, if the viscosity index is less than the above-described lower limit, an energy saving property is decreased, and if it exceeds the above-described upper limit, fluidity at ordinary temperature is decreased and the lubricant base oil according to the present embodiment tends to be not able to be used as a lubricant base oil.

Moreover, the SBV viscosity of the lubricant base oil according to the present embodiment at -20°C is 3,000 to 60,000 mPa·s, preferably 3,000 to 30,000 mPa·s, and more preferably 3,000 to 15,000 mPa·s. If the SBV viscosity at -20°C is less than the above-described lower limit, a sealing property is insufficient, and if it exceeds the above-described upper limit, a low temperature viscosity characteristic is insufficient.

Moreover, the SBV viscosity of the lubricant base oil according to the present embodiment at -30°C is preferably 50,000 to 500,000 mPa·s, more preferably 50,000 to 400,000 mPa·s, and further preferably 50,000 to 300,000 mPa·s. If the SBV viscosity at -25°C is less than the above-described lower limit, a sealing property becomes insufficient, and if it exceeds the above-described upper limit, a low temperature viscosity characteristic becomes insufficient.

Moreover, the kinematic viscosity of the lubricant base oil according to the present embodiment at 40°C is preferably 10 to 20 mm²/s, and more preferably 12 to 16 mm²/s.

Moreover, the freezing point of the lubricant base oil according to the present embodiment is preferably -20 to -5°C, more preferably -18 to -8°C, and further preferably -15 to -10°C. In addition, if the freezing point is less than the above-described lower limit, an energy saving property tends to be decreased, and if it exceeds the above-described upper limit, fluidity at ordinary temperature tends to be decreased and the lubricant base oil according to the present embodiment cannot be used as a lubricant base oil.

Furthermore, in the case of performing a ¹³C-NMR analysis of the lubricant base oil according to the present embodiment, a ratio of CH₂ carbons constituting the main chain to all carbons constituting the lubricant base oil is preferably 15% or more, and more preferably 16% or more. If the ratio is the above-described lower limit or more, a traction coefficient of the lubricant base oil can be decreased (that is, low friction), and it is preferable in terms of an energy saving property.

Furthermore, in the case of performing an FD-MS analysis of the lubricant base oil according to the present embodiment, a cycloparaffin content is preferably 50% or less, and more preferably 40% or less. If the cycloparaffin content is the above-described upper limit or less, abrasion resistance of the lubricant base oil can be further improved.

Moreover, from the viewpoint of improving a low-temperature viscosity characteristic without impairing a viscosity-temperature characteristic at high temperature, the urea adduct value of the lubricant base oil according to the present embodiment is preferably 4% by mass or less, more preferably 3.5% by mass or less, further preferably 3% by mass or less, and particularly preferably 2.5% by mass or less. Furthermore, the urea adduct value of the lubricant base oil may be 0% by mass. However, since a sufficient low-temperature viscosity characteristic and a lubricant base oil having a higher viscosity index can be obtained, and furthermore, dewaxing conditions are loosened to result in excellent economic efficiency, it is preferably 0.1% by mass or more, more preferably 0.5% by mass or more, and particularly preferably 0.8% by mass or more.

Moreover, the content of the saturated content in the lubricant base oil according to the present embodiment is, on the basis of the total amount of the lubricant base oil, preferably 90% by mass or more, more preferably 93% by mass or more, further preferably 95% by mass or more, and particularly preferably 99% by mass or more. The content of the saturated content satisfies the above-described condition so that a viscosity-temperature characteristic and thermal-oxidation stability can be achieved, and furthermore, in the case where an additive agent is blended into the lubricant base oil, the additive agent is sufficiently stably dissolved and maintained in the lubricant base oil and functions of the additive agent can be expressed at a high level. Furthermore, a friction characteristic of the lubricant base oil itself can be improved, and as a result, improvement in a friction-reducing effect and therefore improvement in an energy saving property can be achieved. In addition, the content of the saturated content in the present invention means a value (unit: % by mass) measured in conformity with ASTM D 2007-93.

Moreover, the aromatic content in the lubricant base oil according to the present embodiment is, on the basis of the total amount of the lubricant base oil, preferably 5 % by mass or less, more preferably 0.05 to 3% by mass, further preferably 0.1 to 1% by mass, and particularly preferably 0.1 to 0.5% by mass. If the content of the aromatic content exceeds the above-described upper limit, a viscosity-temperature characteristic, thermal-oxidation stability, a friction characteristic, and furthermore, a volatilization-preventing property, and a low-temperature viscosity characteristic tend to be decreased, and moreover, in the case where an additive agent is blended into the lubricant base oil, an effect of the additive agent tends to be decreased. Furthermore, although the lubricant base oil according to the present embodiment may not contain the aromatic content, solubility of the additive agent can be further increased by making the content of the aromatic content be 0.05% by mass or more.

In addition, the content of the aromatic content in the present invention means a value measured in conformity with ASTM D 2007-93. Generally, the aromatic content includes, in addition to alkylbenzenes and alkylnaphthalenes, anthracene, phenanthrene, alkylated products thereof, and moreover, compounds in which four benzene rings or more are condensed, and aromatic compounds having a hetero atom, such as pyridines, quinolines, phenols, and naphthols.

Furthermore, the content of the sulfur content in the lubricant base oil according to the present embodiment depends on the content of the sulfur content in the raw material. For example, in the case of using a raw material substantially not containing sulfur, such as a synthetic wax constituent obtained by a Fischer-Tropsch reaction or the like, a lubricant base oil substantially not containing sulfur can be obtained. Moreover, in the case of using a raw material containing sulfur, such as slack wax obtained in the refining process of the lubricant base oil and micro wax obtained in the wax refining process, the sulfur content in the obtained lubricant base oil is generally 100 mass ppm or more. In the lubricant base oil of the present invention, in terms of further improvement in thermal-oxidation stability and reduction in the sulfur content, the content of the sulfur content is preferably 10 mass ppm or less, more preferably 5 mass ppm or less, further preferably 3 mass ppm or less, and particularly preferably 1 mass ppm or less.

Furthermore, in terms of cost reduction, slack wax or the like is preferably used as a raw material, and in this case, the sulfur content in the obtained lubricant base oil is preferably 50 mass ppm or less, and more preferably 10 mass ppm or less. In addition, the sulfur content in the present invention means a sulfur content measured in conformity with JIS K 2541-1996.

Moreover, the pour point of the lubricant base oil according to the present embodiment is preferably -5°C or less, more preferably - 10°C or less, and further preferably -12.5°C or less. If the pour point exceeds the above-described upper limit, low temperature fluidity of the entire lubricant oil using the lubricant base oil tends to be decreased. Furthermore, the pour point of the lubricant base oil according to the present embodiment is preferably -20°C or more, more preferably - 17.5°C or more, and further preferably -15°C or more. If the pour point is less than -20°C, it becomes difficult for the SBV viscosity at -20°C to be within a range of 3,000 to 60,000 mPa·s, and a sealing property tends to be insufficient. In addition, the pour point in the present invention means a pour point measured in conformity with JIS K 2269-1987.

Moreover, the CCS viscosity of the lubricant base oil according to the present embodiment at -30°C is preferably 1,500 mPa·s or less, and more preferably 1,200 mPa·s or less. Furthermore, the CCS viscosity of the lubricant base oil at -35°C is preferably 2,500 mPa·s or less, and more preferably 2,000 mPa·s or less. If the CCS viscosity at - 30°C or at -35°C exceeds the above-described upper limit, low temperature fluidity of the entire lubricant oil using the lubricant base oil tends to be decreased. In addition, the CCS viscosity at -30°C or at-35°C means a viscosity measured in conformity with JIS K 2010-1993.

Moreover, the density of the lubricant base oil according to the present embodiment at 15°C (ρ₁₅) is preferably a ρ value represented by the following formula (1) or less, that is ρ₁₅≤ρ. $ρ + 0.0025 \times kv 100 + 0.816$

### [In the formula, kv100 represents kinematic viscosity of lubricant base oil at 100°C (mm²/s).]

In addition, in the case of ρ₁₅>ρ, a viscosity-temperature characteristic, thermal-oxidation stability, and furthermore, a volatilization-preventing property, and a low-temperature viscosity characteristic tend to be decreased, and moreover, in the case where an additive agent is blended into the lubricant base oil, an effect of the additive agent tends to be decreased.

More specifically, ρ₁₅ of the lubricant base oil is preferably 0.815 or less, and more preferably 0.810 or less.

In addition, the density at 15°C in the present invention means a density measured at 15°C in conformity with JIS K 2249-1995.

Moreover, the NOACK evaporation of the lubricant base oil according to the present embodiment is preferably 8% by mass or more, more preferably 9% by mass or more, further preferably 10 or more, and moreover, preferably 15% by mass or less, more preferably 14% by mass or less, and further preferably 13% by mass or less. When the NOACK evaporation is the above-described lower limit, improvement in a low-temperature viscosity characteristic tends to become difficult. Furthermore, the NOACK evaporation exceeding the above-described upper limit is not preferable because, in the case where the lubricant base oil is used for an internal combustion engine lubricant oil or the like, evaporation loss of the lubricant oil is increased, and therefore, catalyst poisoning is accelerated. In addition, the NOACK evaporation in the present invention means evaporation loss measured in conformity with ASTM D 5800-95.

### [Second Embodiment: Lubricant Base Oil that is Hydrocarbon Oil that satisfies Condition (ii)]

The lubricant base oil according to the second embodiment of the present invention is a hydrocarbon oil having a kinematic viscosity at 100°C of 5 to 9 mm²/s and an SBV viscosity at -20°C of 3,000 to 30,000 mPa·s.

In addition, conventionally, a pour point used as an index of a low-temperature viscosity characteristic of a lubricant base oil evaluates ease of flow, that is to say, a bulk viscosity. In contrast, the SBV viscosity in the present invention can evaluate not a bulk viscosity but mobility of a base oil at the molecular level. For example, a lubricant base oil does not flow at a temperature lower than a pour point, but can move at the molecular level due to distortion between molecules constituting the base oil to impart the SBV viscosity. The lubricant base oil according to the present embodiment is made based on the above-described present inventors' knowledge, and has an unexpected significant effect that, in a lubricant base oil having a kinematic viscosity at 100°C of 5 to 9 mm²/s, by making the SBV viscosity at -20°C of the lubricant base oil be 3,000 to 30,000 mPa·s, a sealing property can be improved while sufficiently maintaining a low-temperature viscosity characteristic.

The kinematic viscosity of the lubricant base oil according to the present embodiment at 100°C is 5 to 9 mm²/s, preferably 5.5 to 8.5 mm²/s, and more preferably 6 to 8 mm²/s.

Moreover, the SBV viscosity of the lubricant base oil according to the present embodiment at -20°C is 3,000 to 30,000 mPa·s, preferably 3,000 to 25,000 mPa·s, and more preferably 3,000 to 20,000 mPa·s. If the SBV viscosity at -20°C is less than the above-described lower limit, a sealing property is insufficient, and if it exceeds the above-described upper limit, a low temperature viscosity characteristic is insufficient.

Moreover, the SBV viscosity of the lubricant base oil according to the present embodiment at -25°C is preferably 5,000 to 500,000 mPa·s, more preferably 5,000 to 400,000 mPa·s, and further preferably 5,000 to 300,000 mPa·s. If the SBV viscosity at -25°C is less than the above-described lower limit, a sealing property becomes insufficient, and if it exceeds the above-described upper limit, a low temperature viscosity characteristic becomes insufficient.

Moreover, the kinematic viscosity of the lubricant base oil according to the present embodiment at 40°C is preferably 25 to 40 mm²/s, and more preferably 28 to 35 mm²/s.

Moreover, the viscosity index of the lubricant base oil according to the present embodiment is 155 or more, preferably 157 or more, and more preferably 158 to 165. In addition, if the viscosity index is less than the above-described lower limit, an energy saving property is decreased, and if it exceeds the above-described upper limit, fluidity at ordinary temperature tends to be decreased and the lubricant base oil according to the present embodiment cannot be used as a lubricant base oil.

Moreover, the freezing point of the lubricant base oil according to the present embodiment is preferably -15 to -5°C, more preferably -14 to -7°C, and further preferably -13 to -8°C. In addition, if the freezing point is less than the above-described lower limit, an energy saving property tends to be decreased, and if it exceeds the above-described upper limit, fluidity at ordinary temperature tends to be decreased and the lubricant base oil according to the present embodiment cannot be used as a lubricant base oil.

Furthermore, in the case of performing a ¹³C-NMR analysis of the lubricant base oil according to the present embodiment, a ratio of CH₂ carbons constituting the main chain to all carbons constituting the lubricant base oil is preferably 20% or more, and more preferably 18% or more. If the ratio is the above-described lower limit or more, a traction coefficient of the lubricant base oil can be decreased (that is, low friction), and it is preferable in terms of an energy saving property.

Furthermore, in the case of performing an FD-MS analysis of the lubricant base oil according to the present embodiment, a cycloparaffin content is preferably 60% or less, and more preferably 65% or less. If the cycloparaffin content is the above-described upper limit or less, abrasion resistance of the lubricant base oil can be further improved.

Moreover, from the viewpoint of improving a low-temperature viscosity characteristic without impairing a viscosity-temperature characteristic at high temperature, the urea adduct value of the lubricant base oil according to the present embodiment is preferably 4% by mass or less, more preferably 3.5% by mass or less, further preferably 3% by mass or less, and particularly preferably 2.5% by mass or less. Furthermore, the urea adduct value of the lubricant base oil may be 0% by mass. However, since a sufficient low-temperature viscosity characteristic and a lubricant base oil having a higher viscosity index can be obtained, and furthermore, dewaxing conditions are loosened to result in excellent economic efficiency, it is preferably 0.1% by mass or more, more preferably 0.5% by mass or more, and particularly preferably 0.8% by mass or more.

Moreover, the content of the saturated content in the lubricant base oil according to the present embodiment is, on the basis of the total amount of the lubricant base oil, preferably 90% by mass or more, more preferably 93% by mass or more, further preferably 95% by mass or more, and particularly preferably 99% by mass or more. The content of the saturated content satisfies the above-described condition so that a viscosity-temperature characteristic and thermal-oxidation stability can be achieved, and furthermore, in the case where an additive agent is blended into the lubricant base oil, the additive agent is sufficiently stably dissolved and maintained in the lubricant base oil and functions of the additive agent can be expressed at a high level. Furthermore, a friction characteristic of the lubricant base oil itself can be improved, and as a result, improvement in a friction-reducing effect and therefore improvement in an energy saving property can be achieved.

Moreover, the aromatic content in the lubricant base oil according to the present embodiment is, on the basis of the total amount of the lubricant base oil, preferably 5% by mass or less, more preferably 0.05 to 3% by mass, further preferably 0.1 to 1% by mass, and particularly preferably 0.1 to 0.5% by mass. If the content of the aromatic content exceeds the above-described upper limit, a viscosity-temperature characteristic, thermal-oxidation stability, a friction characteristic, and furthermore, a volatilization-preventing property, and a low-temperature viscosity characteristic tend to be decreased, and moreover, in the case where an additive agent is blended into the lubricant base oil, an effect of the additive agent tends to be decreased. Furthermore, although the lubricant base oil according to the present embodiment may not contain the aromatic content, solubility of the additive agent can be further increased by making the content of the aromatic content be 0.05% by mass or more.

Furthermore, the content of the sulfur content in the lubricant base oil according to the present embodiment depends on the content of the sulfur content in the raw material. For example, in the case of using a raw material substantially not containing sulfur, such as a synthetic wax constituent obtained by a Fischer-Tropsch reaction or the like, a lubricant base oil substantially not containing sulfur can be obtained. Moreover, in the case of using a raw material containing sulfur, such as slack wax obtained in the refining process of the lubricant base oil and micro wax obtained in the wax refining process, the sulfur content in the obtained lubricant base oil is generally 100 mass ppm or more. In the lubricant base oil of the present invention, in terms of further improvement in thermal-oxidation stability and reduction in the sulfur content, the content of the sulfur content is preferably 10 mass ppm or less, more preferably 5 mass ppm or less, further preferably 3 mass ppm or less, and particularly preferably 1 mass ppm or less.

Furthermore, in terms of cost reduction, slack wax or the like is preferably used as a raw material, and in this case, the sulfur content in the obtained lubricant base oil is preferably 50 mass ppm or less, and more preferably 10 mass ppm or less.

Moreover, the pour point of the lubricant base oil according to the present embodiment is preferably -5°C or less, more preferably - 10°C or less, and further preferably -12.5°C or less. If the pour point exceeds the above-described upper limit, low temperature fluidity of the entire lubricant oil using the lubricant base oil tends to be decreased. Furthermore, the pour point of the lubricant base oil according to the present embodiment is preferably -20°C or more, more preferably - 17.5°C or more, and further preferably -15°C or more. If the pour point is less than -20°C, it becomes difficult for the SBV viscosity at -20°C to be within a range of 3,000 to 30,000 mPa·s, and a sealing property tends to be insufficient.

Moreover, the CCS viscosity of the lubricant base oil according to the present embodiment at -30°C is preferably 950 mPa·s or less, and more preferably 900 mPa·s or less. Furthermore, the CCS viscosity of the lubricant base oil at -35°C is preferably 1,600 mPa·s or less, and more preferably 1,500 mPa·s or less. If the CCS viscosity at-30°C or at -35°C exceeds the above-described upper limit, low temperature fluidity of the entire lubricant oil using the lubricant base oil tends to be decreased.

Moreover, the density of the lubricant base oil according to the present embodiment at 15°C (ρ₁₅) is preferably a ρ value represented by the following formula (1) or less, that is ρ₁₅≤ρ. $ρ = 0.0025 \times kv 100 + 0.816$

### [In the formula, kv100 represents kinematic viscosity of lubricant base oil at 100°C (mm²/s).]

In addition, in the case of ρ₁₅>ρ, a viscosity-temperature characteristic, thermal-oxidation stability, and furthermore, a volatilization-preventing property, and a low-temperature viscosity characteristic tend to be decreased, and moreover, in the case where an additive agent is blended into the lubricant base oil, an effect of the additive agent tends to be decreased.

More specifically, ρ₁₅ of the lubricant base oil is preferably 0.830 or less, and more preferably 0.825 or less.

### [Third Embodiment: Lubricant Base Oil that is Hydrocarbon Oil that satisfies Condition (iii)]

The lubricant base oil according to the third embodiment of the present invention is a lubricant base oil that is a hydrocarbon oil having a kinematic viscosity at 100°C of 2.0 to 3.0 mm²/s, a viscosity index of 130 or more, a pour point of -27.5°C or more, and an SBV viscosity at-30°C of 1,000 to 30,000 mPa·s.

In addition, conventionally, a pour point used as an index of a low-temperature viscosity characteristic of a lubricant base oil evaluates ease of flow, that is to say, a bulk viscosity. In contrast, the SBV viscosity in the present invention can evaluate not a bulk viscosity but mobility of a base oil at the molecular level. For example, a lubricant base oil does not flow at a temperature lower than a pour point, but can move at the molecular level due to distortion between molecules constituting the base oil to impart the SBV viscosity. The lubricant base oil according to the present embodiment is made based on the above-described present inventors' knowledge, and has an unexpected significant effect that, in a lubricant base oil having a kinematic viscosity at 100°C of 2.0 to 3.0 mm²/s and a viscosity index of 130 or more, by making the SBV viscosity at -30°C of the lubricant base oil be 1,000 to 30,000 mPa·s, a sealing property can be improved while sufficiently maintaining a low-temperature viscosity characteristic.

The kinematic viscosity of the lubricant base oil according to the present embodiment at 100°C is 2.0 to 3.0 mm²/s, preferably 2.1 to 2.9 mm²/s, and more preferably 2.2 to 2.8 mm²/s.

Moreover, the viscosity index of the lubricant base oil according to the present embodiment is 130 or more, preferably 131 or more, and more preferably 132 to 140. If the viscosity index is less than the above-described lower limit, an energy saving property is decreased, and if it exceeds the above-described upper limit, fluidity at ordinary temperature is decreased and the lubricant base oil according to the present embodiment cannot be used as a lubricant base oil.

Moreover, the SBV viscosity of the lubricant base oil according to the present embodiment at -30°C is 1,000 to 30,000 mPa·s, preferably 1,000 to 20,000 mPa·s, and more preferably 1,000 to 15,000 mPa·s. If the SBV viscosity at -30°C is less than the above-described lower limit, a sealing property is insufficient, and if it exceeds the above-described upper limit, a low temperature characteristic is insufficient.

Moreover, the SBV viscosity of the lubricant base oil according to the present embodiment at -35°C is preferably 3,000 to 500,000 mPa·s, more preferably 3,000 to 400,000 mPa·s, and further preferably 3,000 to 300,000 mPa·s. If the SBV viscosity at -35°C is less than the above-described lower limit, a sealing property is insufficient, and if it exceeds the above-described upper limit, a low-temperature viscosity characteristic is insufficient.

Moreover, the SBV viscosity of the lubricant base oil according to the present embodiment at -40°C is preferably 5,000 to 750,000 mPa·s, more preferably 5,000 to 500,000 mPa·s, and further preferably 5,000 to 400,000 mPa·s. If the SBV viscosity at -40°C is less than the above-described lower limit, a sealing property is insufficient, and if it exceeds the above-described upper limit, a low-temperature viscosity characteristic is insufficient.

Moreover, the kinematic viscosity of the lubricant base oil according to the present embodiment at 40°C is preferably 7 to 12 mm²/s, and more preferably 8 to 10 mm²/s.

Moreover, the freezing point of the lubricant base oil according to the present embodiment is preferably -30 to -10°C, more preferably -29 to -15°C, and further preferably -28 to -20°C. In addition, if the freezing point is less than the above-described lower limit, an energy saving property tends to be decreased, and if it exceeds the above-described upper limit, fluidity at ordinary temperature tends to be decreased and the lubricant base oil according to the present embodiment cannot be used as a lubricant base oil.

Furthermore, in the case of performing a ¹³C-NMR analysis of the lubricant base oil according to the present embodiment, a ratio of CH₂ carbons constituting the main chain to all carbons constituting the lubricant base oil is preferably 15% or more, and more preferably 15% or more. If the ratio is the above-described lower limit or more, a traction coefficient of the lubricant base oil can be decreased (that is, low friction), and it is preferable in terms of an energy saving property.

Furthermore, in the case of performing an FD-MS analysis of the lubricant base oil according to the present embodiment, a cycloparaffin content is preferably 30% or less, and more preferably 25% or less. If the cycloparaffin content is the above-described upper limit or less, abrasion resistance of the lubricant base oil can be further improved.

Moreover, from the viewpoint of improving a low-temperature viscosity characteristic without impairing a viscosity-temperature characteristic at high temperature, the urea adduct value of the lubricant base oil according to the present embodiment is preferably 4% by mass or less, more preferably 3.5% by mass or less, further preferably 3% by mass or less, and particularly preferably 2.5% by mass or less. Furthermore, the urea adduct value of the lubricant base oil may be 0% by mass. However, since a sufficient low-temperature viscosity characteristic and a lubricant base oil having a higher viscosity index can be obtained, and furthermore, dewaxing conditions are loosened to result in excellent economic efficiency, it is preferably 0.1% by mass or more, more preferably 0.5% by mass or more, and particularly preferably 0.8% by mass or more.

Moreover, the content of the saturated content in the lubricant base oil according to the present embodiment is, on the basis of the total amount of the lubricant base oil, preferably 90% by mass or more, more preferably 93% by mass or more, further preferably 95% by mass or more, and particularly preferably 99% by mass or more. The content of the saturated content satisfies the above-described condition so that a viscosity-temperature characteristic and thermal-oxidation stability can be achieved, and furthermore, in the case where an additive agent is blended into the lubricant base oil, the additive agent is sufficiently stably dissolved and maintained in the lubricant base oil and functions of the additive agent can be expressed at a high level. Furthermore, a friction characteristic of the lubricant base oil itself can be improved, and as a result, improvement in a friction-reducing effect and therefore improvement in an energy saving property can be achieved.

Moreover, the aromatic content in the lubricant base oil according to the present embodiment is, on the basis of the total amount of the lubricant base oil, preferably 5% by mass or less, more preferably 0.05 to 3% by mass, further preferably 0.1 to 1% by mass, and particularly preferably 0.1 to 0.5% by mass. If the content of the aromatic content exceeds the above-described upper limit, a viscosity-temperature characteristic, thermal-oxidation stability, a friction characteristic, and furthermore, a volatilization-preventing property, and a low-temperature viscosity characteristic tend to be decreased, and moreover, in the case where an additive agent is blended into the lubricant base oil, an effect of the additive agent tends to be decreased. Furthermore, although the lubricant base oil according to the present embodiment may not contain the aromatic content, solubility of the additive agent can be further increased by making the content of the aromatic content be 0.05% by mass or more.

Furthermore, the content of the sulfur content in the lubricant base oil according to the present embodiment depends on the content of the sulfur content in the raw material. For example, in the case of using a raw material substantially not containing sulfur, such as a synthetic wax constituent obtained by a Fischer-Tropsch reaction or the like, a lubricant base oil substantially not containing sulfur can be obtained. Moreover, in the case of using a raw material containing sulfur, such as slack wax obtained in the refining process of the lubricant base oil and micro wax obtained in the wax refining process, the sulfur content in the obtained lubricant base oil is generally 100 mass ppm or more. In the lubricant base oil of the present invention, in terms of further improvement in thermal-oxidation stability and reduction in the sulfur content, the content of the sulfur content is preferably 10 mass ppm or less, more preferably 5 mass ppm or less, further preferably 3 mass ppm or less, and particularly preferably 1 mass ppm or less.

Furthermore, in terms of cost reduction, slack wax or the like is preferably used as a raw material, and in this case, the sulfur content in the obtained lubricant base oil is preferably 50 mass ppm or less, and more preferably 10 mass ppm or less.

Moreover, the pour point of the lubricant base oil according to the present embodiment is preferably -5°C or less, more preferably-12.5°C or less, and further preferably -15°C or less. If the pour point exceeds the above-described upper limit, low temperature fluidity of the entire lubricant oil using the lubricant base oil tends to be decreased. Furthermore, the pour point of the lubricant base oil according to the present embodiment is -27.5°C or more, and preferably -25°C or more. If the pour point is less than -27.5°C, it becomes difficult for the SBV viscosity at -20°C to be within a range of 3,000 to 60,000 mPa·s, and a sealing property tends to be insufficient.

Moreover, the CCS viscosity of the lubricant base oil according to the present embodiment at -30°C is preferably 1,000 mPa·s or less, and more preferably 750 mPa·s or less. Furthermore, the CCS viscosity of the lubricant base oil at -35°C is preferably 1,300 mPa·s or less, and more preferably 1,000 mPa·s or less. If the CCS viscosity at-30°C or at -35°C exceeds the above-described upper limit, low temperature fluidity of the entire lubricant oil using the lubricant base oil tends to be decreased.

Moreover, the density of the lubricant base oil according to the present embodiment at 15°C (ρ₁₅) is preferably a ρ value represented by the following formula (1) or less, that is ρ₁₅≤ρ. $ρ = 0.0025 \times kv 100 + 0.816$

### [In the formula, kv100 represents kinematic viscosity of lubricant base oil at 100°C (mm²/s).]

In addition, in the case of ρ₁₅>ρ, a viscosity-temperature characteristic, thermal-oxidation stability, and furthermore, a volatilization-preventing property, and a low-temperature viscosity characteristic tend to be decreased, and moreover, in the case where an additive agent is blended into the lubricant base oil, an effect of the additive agent tends to be decreased.

More specifically, ρ₁₅ of the lubricant base oil is preferably 0.806 or less, and more preferably 0.8058 or less.

Moreover, the NOACK evaporation of the lubricant base oil according to the present embodiment is preferably 20% by mass or more, more preferably 25% by mass or more, further preferably 30 or more, and moreover, preferably 50% by mass or less, more preferably 48% by mass or less, and further preferably 46% by mass or less. When the NOACK evaporation is the above-described lower limit, improvement in a low-temperature viscosity characteristic tends to become difficult. Furthermore, the NOACK evaporation exceeding the above-described upper limit is not preferable because, in the case where the lubricant base oil is used for an internal combustion engine lubricant oil or the like, evaporation loss of the lubricant oil is increased, and therefore, catalyst poisoning is accelerated.

The lubricant base oils according to the above-described first to third embodiments excel in a low-temperature viscosity characteristic and a sealing property, and can be suitably used as lubricant base oils for various applications. Specifically, examples of the applications of the lubricant base oil include lubricant oils used for internal combustion engines such as passenger vehicle gasoline engines, two-wheel vehicle gasoline engines, diesel engines, gas engines, gas heat pump engines, marine engines, and power-generating engines (internal combustion engine lubricant oil), lubricant oils used for driving transmission devices such as automatic transmissions, manual transmissions, non-stage transmissions, and final reduction gears (driving transmission device oil), hydraulic oils used for hydraulic systems such as dampers and construction machines, compressor oils, turbine oils, industrial gear oils, refrigerant oils, rust preventing oils, heating medium oils, gas holder seal oils, bearing oils, paper machine oils, machine tool oils, sliding guide surface oils, electrical insulating oils, cutting oils, press oils, rolling oils, and heat treating oils, and by using the lubricant base oil according to the present embodiment for these applications, both a low-temperature viscosity characteristic and a sealing property can be satisfied at a high level.

In the above-described applications, the lubricant base oil according to each embodiment may be used alone, or the lubricant base oil according to each embodiment may be used in combination with one, or two or more other base oils. In addition, when the lubricant base oil according to each embodiment is used in combination with other base oils, a ratio of the lubricant base oil of the present invention in the mixed-base oil is preferably 30% by mass or more, more preferably 50% by mass or more, and further preferably 70% by mass or more.

Other base oils used in combination with the lubricant base oil according to each embodiment are not particularly limited, and examples of mineral base oils include solvent refined mineral oils, hydrocracked mineral oils, hydrorefined mineral oils, and solvent dewaxed base oils having a kinematic viscosity at 100°C of 1 to 100 mm²/s, for example.

Moreover, examples of synthetic base oils include poly-α-olefins or hydrides thereof, isobutene oligomers or hydrides thereof, isoparaffins, alkylbenzenes, alkylnaphthalenes, diesters (ditridecyl glutarate, di-2-ethylhexyl adipate, diisodecyl adipate, ditridecyl adipate, di-2-ethylhexyl sebacate and the like), polyol esters (trimethylolpropane caprylate, trimethylolpropane pelargonate, pentaerythritol 2-ethylhexanoate, pentaerythritol pelargonate and the like), polyoxyalkylene glycols, dialkyldiphenyl ethers, and polyphenyl ethers, and among them, poly-α-olefins are preferable. Typically, examples of the poly-α-olefins include α-olefin oligomers or co-oligomers having a carbon number of 2 to 32, and preferably 6 to 16 (1-octene oligomer, decene oligomer, ethylene-propylene co-oligomer and the like) and hydrides thereof.

Although a producing method of poly-α-olefins is not particularly limited, examples thereof include a method in which α-olefin is polymerized in the presence of a polymerization catalyst such as a Friedel-Crafts catalyst including a complex of aluminum trichloride or boron trifluoride with water, an alcohol (ethanol, propanol, butanol and the like), a carboxylic acid, or ester.

Furthermore, various additive agents may be blended into the lubricant base oil according to each embodiment or the mixed-base oil of the lubricant base oil and other lubricant base oils, if necessary. Such additive agents are not particularly limited, and arbitrary additive agents that are conventionally used in the field of lubricant oils can be blended. Specifically, examples of the lubricant oil additive agents include antioxidants, ashless dispersants, metal-based detergents, extreme pressure agents, antiwear agents, viscosity index improvers, pour-point depressants, friction modifiers, oiliness agents, corrosion inhibitors, rust-preventive agents, demulsifying agents, metal deactivating agents, seal swelling agents, antifoaming agents, and coloring agents. These additive agents may be used singly or two or more kinds thereof may be used in combination.

For example, the lubricant base oil according to each embodiment can effectively exhibit the addition effect of a pour-point depressant. Therefore, when the lubricant base oil according to each embodiment or the mixed-base oil of the lubricant base oil and other lubricant base oils contains a pour-point depressant, an excellent low-temperature viscosity characteristic (MRV viscosity at -40°C is preferably 20,000 mPa·s or less, more preferably 15,000 mPa·s or less, and further preferably 10,000 mPa·s or less) can be achieved. In addition, the MRV viscosity at -40°C described in the present invention means an MRV viscosity at -40°C measured in conformity with JPI-5S-42-93.

Further, when a pour-point depressant is blended into the lubricant base oil according to the first embodiment or the lubricant base oil according to the second embodiment, the MRV viscosity at -40°C can be 12,000 mPa·s or less, and a lubricant oil composition having an extremely excellent low-temperature viscosity characteristic of more preferably 10,000 mPa·s or less, further preferably 8,000 mPa·s, and particularly preferably 6,500 mPa·s or less can be obtained. In this case, the amount of the pour-point depressant blended is, on the basis of the total amount of the composition, 0.05 to 2% by mass, and preferably 0.1 to 1.5% by mass, in particular, in terms of capable of decreasing the MRV viscosity, the range of 0.15 to 0.8% by mass is the best, as the pour-point depressant, one having the weight-average molecular weight of preferably 10,000 to 300,000, and more preferably 50,000 to 200,000 is particularly preferable, and moreover, as the pour-point depressant, polymethacrylate-based one is particularly preferable.

### Examples

Hereinafter, the present invention will be described more specifically based on examples and comparative examples, but the present invention is not limited to the following examples.

### [Examples 1-1 to 1-3, Comparative Examples 1-1 and 1-2]

In Examples 1-1 to 1-3 and Comparative Examples 1-1 and 1-2, lubricant base oils shown in Table 1 were each prepared. The lubricant base oils in Examples 1-1 to 1-3 are obtained based on the method for producing a lubricant base oil according to the above-described fourth embodiment. In contrast, the lubricant base oils in Comparative Examples 1-1 and 1-2 are obtained by the conventional method for producing a lubricant base oil. Various characteristics of the respective base oils, and the traction coefficients measured under conditions of a load of 50 N (average hertz pressure 0.60 GPa), a sample oil temperature of 50°C, a circumferential velocity of 1 m/s, and a slip ratio of 3%, and using a 27.4 mm steel ball and a steel disc are shown in Table 1.

**[Table 1]**

| Raw materials | Example 1-1 | Example 1-2 | Example 1-3 | Comp. Example 1-1 | Comp. Example 1-2 |
|---|---|---|---|---|---|
| General physical properties | | | | | |
| Density, g/cm³ | 0.8182 | 0.8181 | 0.8083 | 0.8180 | 0.8184 |
| Flash point, °C | 232 | 234 | 228 | 238 | 220 |
| Kinematic viscosity, mm²/s (40°C) | 16.6 | 17.0 | 17.1 | 16.9 | 17.0 |
| (100°C) | 4.09 | 4.13 | 4.10 | 4.16 | 4.10 |
| Viscosity index | 154 | 151 | 146 | 157 | 141 |
| Pour point, °C | -5 | -12.5 | -17.5 | -2.5 | -25 |
| Freezing point, °C | -5 | -15 | -20 | -4 | -26 |
| NOACK, mass% (250°C) | 11.5 | 12.0 | 12.8 | 12.2 | 11.8 |
| Sulfur content, mass ppm | <1 | <1 | <1 | <1 | <1 |
| Chromatography analysis | | | | | |
| Saturated content, mass% | 99.4 | 99.3 | 99.5 | 99.4 | 99.6 |
| Resin content, mass% | 0.4 | 0.3 | 0.2 | 0.4 | 0.2 |
| Aromatic content, mass% | 0.2 | 0.4 | 0.3 | 0.3 | 0.2 |
| Recovery rate, mass% | 100 | 100 | 100 | 100 | 100 |

| Urea adduct | | | | | |
|---|---|---|---|---|---|
| Adduct amount, mass% | 3.18 | 2.72 | 2.08 | 4.05 | 1.15 |

| Low-temperature characteristics | | | | | |
|---|---|---|---|---|---|
| CCS viscosity (-30°C), mPa·s | 870 | 880 | 630 | 990 | 141 |
| (-35°C), mP·s | 1,650 | 1,600 | 1,590 | 1,950 | 1,530 |
| SBV viscosity (-20°C), mPa·s | 57,600 | 12,000 | 3,200 | 62,000 | 810 |
| (-30°C), mPa·s | 478,000 | 156,000 | 51,000 | 880,000 | 3,370 |
| (-35°C), mPa·s | 783,000 | 492,000 | 118,000 | >1,000,000 | 9,150 |

| ¹³C-NMR | | | | | |
|---|---|---|---|---|---|
| CH | 6.6 | 6.8 | 7.2 | 6.4 | 7.4 |
| CH2 | 79,1 | 78.8 | 78.3 | 79.5 | 78.1 |
| CH3 | 14.3 | 14.4 | 14.5 | 14.1 | 14.5 |
| CH2 main chain | 19.8 | 18.6 | 15.2 | 22.0 | 14.7 |

| EI-MS | | | | | |
|---|---|---|---|---|---|
| Paraffins | 92.2 | 92.3 | 92.1 | 92.0 | 92.8 |
| Monocyclic cycloparaffin | 3.8 | 4.5 | 4.2 | 4.6 | 4.0 |
| Bicyclic cycloparaffin | 3.1 | 2.3 | 2.7 | 2.3 | 2.5 |
| Tricyclic cycloparaffin | 0.3 | 0.2 | 0.1 | 0.3 | 0.2 |
| Tetracyclic cycloparaffin | 0.0 | 0.0 | 0.0 | 0.2 | 0.0 |
| Pentacyclic cycloparaffin | 0.2 | 0.1 | 0.1 | 0.0 | 0.1 |
| Hexacyclic cycloparaffin | 0.4 | 0.6 | 0.5 | 0.6 | 0.4 |
| Alkylbenzenes | 0.0 | 0.0 | 0.0 | 0.0 | 0.0 |

| FD-MS | | | | | |
|---|---|---|---|---|---|
| Paraffins | 61.1 | 58.1 | 50.2 | 65.3 | 65.2 |
| Monocyclic cycloparaffin | 31.4 | 34.6 | 39.9 | 28.5 | 29.2 |
| Bicyclic cycloparaffin | 6.3 | 6.6 | 7.1 | 5.5 | 4.4 |
| Tricyclic cycloparaffin | 0.5 | 0.6 | 2.3 | 0.4 | 0.4 |
| Tetracyclic cycloparaffin | 0.3 | 0.0 | 0.2 | 0.0 | 0.0 |
| Pentacyclic cycloparaffin | 0.1 | 0.0 | 0.0 | 0.0 | 0.0 |
| Hexacyclic cycloparaffin | 0.3 | 0.1 | 0.3 | 0.3 | 0.8 |

| Traction coefficient | | | | | |
|---|---|---|---|---|---|
| 50N, 50°C, 1m/s, Slip ratio 3% | 0.012 | 0.013 | 0.015 | 0.011 | 0.018 |

### [Examples 1-4 to 1-9, Comparative Examples 1-3 to 1-5]

In Examples 1-4, 1-6, and 1-8, and Comparative Examples 1-3 and 1-5, the lubricant base oils of Examples 1-1 to 1-3, or Comparative Examples 1-1 and 1-2, respectively, were used as a sample oil. Furthermore, in Examples 1-5, 1-7, and 1-9, and Comparative Examples 1-4 and 1-6, lubricant oil compositions were prepared by adding 10% by mass of a package additive (breakdown: 40% by mass of ashless dispersant, 40% by mass of metal-based detergent, 10% by mass of antiwear agent, 8 % by mass of antioxidant, and 2% by mass of metal deactivating agent) and 5% by mass of a viscosity index improver (polymethacrylate-based, Mw 350,000, effective concentration 50%) to the respective lubricant base oils of Examples 1-1 to 1-3 or Comparative Examples 1-1 and 1-2, respectively, to be used as a sample oil. Moreover, as Comparative Example 1-7, a commercial 0W-20 oil was prepared. The kinematic viscosities and the viscosity indexes of the respective lubricant oil compositions are shown in Table 2.

### [Oil Leakage Test]

With respect to the sample oils of Examples 1-4 to 1-9, and Comparative Examples 1-3 to 1-6, an oil leakage test was performed according to the following procedure.

100 ml of the sample oil is charged in a 200 ml autoclave and an NBR packing is used to be assembled with a tightening torque of 250 N·m using a torque wrench. A two-way cock is used at the upper part and, as a sealing material, a teflon (registered trademark) packing is used to be assembled with a tightening torque of 250 N·m using a torque wrench. After assembling, a pressure is increased to 200 kPa with nitrogen gas. The respective sample oils are subjected to the same operation and are set upside down in a low-temperature thermostat bath that is controlled to be -30±1C°. Results are evaluated by oil leakage from the NBR packing after 48 hours, and with leakage is evaluated as presence and without leakage is evaluated as absence.

The obtained results are shown in Tables 2 and 3.

### [JC08 Hot Mode Fuel Consumption Evaluation Test]

With respect to the lubricant oil compositions of Examples 1-5, 1-7, and 1-9, and Comparative Examples 1-4 and 1-6, a JC08 hot mode fuel consumption evaluation test was performed according to the following procedure.

JC08 mode is a method for measuring fuel consumption of vehicles, established by Ministry of Land, Infrastructure, Transport and Tourism (for details, refer to Ministry of Land, Infrastructure, Transport and Tourism, Announcement that Prescribes Details of Safety Standards for Road Trucking Vehicles [2009.07.30] Attachment 42 Measurement Method of Exhaust Gas of Light and Middle Vehicles). JC08 is classified into a cold mode that starts in an engine cold state and a hot mode that measures fuel consumption in an engine warm state. In the test, a 2.5 L, FF gasoline engine vehicle (Toyota ESTIMA) was selected, the engine was washed and filled with a newly-prepared sample oil before the start of the test, the test vehicle was made to warm up at a constant rate of 60±2 km/h for 15 minutes or more on a chassis dynamometer, and then, was quickly returned to the idling state, the vehicle was driven in a predetermined running pattern, and consumed fuel was calculated from exhaust gas to determine fuel consumption. The obtained results are shown in Tables 2 and 3.

**[Table 2]**

| | | Example 1-4 | Example 1-5 | Example 1-6 | Example 1-7 | Example 1-8 | Example 1-9 |
|---|---|---|---|---|---|---|---|
| Base oil | Kind | Example 1 | Example 1 | Example 2 | Example 2 | Example 3 | Example 3 |
| | Content (% by mass) | 100 | Balance | 100 | Balance | Balance | Balance |
| Package additive (% by mass) | | - | 10 | - | 10 | - | 10 |
| Viscosity index improver (% by mass) | | - | 5 | - | 5 | - | 5 |
| Characteristics of sample oil (0W -20) | | | | | | | |
| Kinematic viscosity, mm²/s (100°C) | | 4.09 | 8.19 | 4.13 | 8.22 | 4.10 | 8.18 |
| Viscosity index | | 154 | 244 | 151 | 240 | 146 | 242 |
| SBV viscosity (mPa·s) | | | | | | | |
| -20°C | | 57,600 | 59,000 | 3,200 | 3,450 | 3,200 | 3,380 |
| -30°C | | 478,000 | 520,000 | 51,000 | 53,000 | 51,000 | 52,000 |
| Oil leakage test (-20°C) | | | | | | | |
| Presence or absence of leakage | | Absence | Absence | Absence | Absence | Absence | Absence |
| JC08 hot mode fuel consumption | | | | | | | |
| Fuel consumption improving ratio, % | | - | 1.85 | - | 1.71 | - | 1.52 |

**[Table 3]**

| | | Comp. Example 1-3 | Comp. Example 1-4 | Comp. Example 1-5 | Comp. Example 1-6 | Comp. Example 1-7 |
|---|---|---|---|---|---|---|
| Base oil | Kind | Comp. Example 1 | Comp. Example 1 | Comp. Example 2 | Comp. Example 2 | Commercial 0W-20 oil |
| | Content (mass%) | 100 | Balance | 100 | Balance | |
| Package additive (mass%) | | - | 10 | - | 10 | |
| Viscosity index improver (mass%) | | - | 5 | - | 5 | |
| Characteristics of sample oil (0W-20) | | | | | | |
| Kinematic viscosity, mm²/s (100°C) | | 4.16 | 8.28 | 4.04 | 8.33 | 8.42 |
| viscosity index | | 157 | 245 | 141 | 237 | 230 |
| SBV viscosity (mPa·s) | | | | | | |
| -20°C | | 62,000 | 68,000 | 810 | 3,500 | - |
| -30°C | | 880,000 | >1,000,000 | 3,370 | 4,800 | - |
| Oil leakage test (-20°C) Presence or absence of leakage | | Absence | Absence | Presence | Presence | - |
| JC08 hot mode fuel consumption Fuel consumption improving ratio, % | | - | 0.11 | - | 0.05 | - |

### [Examples 2-1 and 2-2, Comparative Examples 2-1 to 2-3]

In Examples 2-1 and 2-2 and Comparative Examples 2-1 to 2-3, lubricant base oils shown in Table 4 were each prepared. The lubricant base oils in Examples 2-1 and 2-2 are obtained based on the method for producing a lubricant base oil according to the above-described fourth embodiment. In contrast, the lubricant base oils in Comparative Examples 2-1 to 2-3 are obtained by the conventional method for producing a lubricant base oil. Various characteristics of the respective base oils, and the traction coefficients measured under conditions of a load of 50 N (average hertz pressure 0.60 GPa), a sample oil temperature of 50°C, a circumferential velocity of 1 m/s, and a slip ratio of 3%, and using a 27.4 mm steel ball and a steel disc are shown in Table 4.

**[Table 4]**

| Raw materials | Example 2-1 | Example 2-2 | Comp. Example 2-1 | Comp. Example 2-2 | Comp. Example 2-3 |
|---|---|---|---|---|---|
| General physical properties | | | | | |
| Density, g/cm³ | 0.8273 | 0.8272 | 0.8270 | 0.8260 | 0.8288 |
| Flash point, °C | 262 | 260 | 264 | 250 | 254 |
| Kinematic viscosity, mm²/s (40°C) | 30.3 | 28.2 | 29.4 | 26.0 | 30.8 |
| (100°C) | 6.30 | 5.92 | 6.20 | 5.48 | 6.07 |
| Viscosity index | 165 | 162 | 167 | 154 | 148 |
| Pour point, °C | -5 | -12.5 | -2.5 | -15 | -30 |
| Freezing point, °C | -5 | -14 | -4 | -17 | -32 |
| Sulfur content, mass ppm | <1 | <1 | <1 | <1 | <1 |
| Chromatography analysis | | | | | |
| Saturated content, mass% | 99.2 | 99.2 | 99.3 | 99.5 | 99.4 |
| Resin content, mass% | 0.4 | 0.3 | 0.3 | 0.2 | 0.2 |
| Aromatic content, mass% | 0.4 | 0.5 | 0.4 | 0.3 | 0.4 |
| Recovery rate, mass% | 100 | 100 | 100 | 100 | 100 |

| Urea adduct | | | | | |
|---|---|---|---|---|---|
| Adduct amount, mass% | 1.25 | 0.77 | 2.33 | 0.11 | 0.13 |
| Low-temperature characteristics | | | | | |
| CCS viscosity (-30°C), mPa·s | 790 | 880 | 1,070 | 995 | 1,020 |
| (-35°C), mP·s | 1,210 | 1,320 | 1,780 | 1,625 | 1,850 |
| SBV viscosity (-20°C), mP·s | 29,000 | 3,200 | 122,000 | 2,100 | 1,030 |
| (-25°C), mP·s | 470,000 | 5,300 | >1,000,000 | 4,300 | 1,700 |

| ¹³C-NMR | | | | | |
|---|---|---|---|---|---|
| CH | 6.2 | 6.5 | 6.0 | 7.1 | 6.8 |
| CH2 | 82.0 | 81.5 | 83.2 | 79.8 | 80.0 |
| CH3 | 11.2 | 12.0 | 10.8 | 13.1 | 13.2 |
| CH2 main chain | 25.3 | 20.3 | 25.9 | 18.0 | 16.0 |

| EI-MS | | | | | |
|---|---|---|---|---|---|
| Paraffins | 81.2 | 80.1 | 82.6 | 83.2 | 80.0 |
| Monocyclic cycloparaffin | 12.9 | 13.4 | 11.8 | 11.0 | 12.7 |
| Bicyclic cycloparaffin | 4.8 | 5.0 | 3.9 | 4.3 | 5.3 |
| Tricyclic cycloparaffin | 0.9 | 1.0 | 0.8 | 0.6 | 1.1 |
| Tetracyclic cycloparaffin | 0.1 | 0.1 | 0.1 | 0.1 | 0.2 |
| Pentacyclic cycloparaffin | 0.0 | 0.0 | 0.2 | 0.2 | 0.2 |
| Hexacyclic cycloparaffin | 0.1 | 0.4 | 0.6 | 0.6 | 0.5 |
| Alkylbenzenes | 0.0 | 0.0 | 0.0 | 0.0 | 0.0 |

| FD-MS | | | | | |
|---|---|---|---|---|---|
| Paraffins | 36.8 | 39.7 | 35.9 | 47.2 | 49.4 |
| Monocyclic cycloparaffin | 46.9 | 44.1 | 47.2 | 41.2 | 39.5 |
| Bicyclic cycloparaffin | 13.8 | 13.0 | 14.1 | 9.7 | 8.7 |
| Tricyclic cycloparaffin | 2.1 | 2.4 | 2.2 | 1.4 | 1.2 |
| Tetracyclic cycloparaffin | 0.1 | 0.2 | 0.2 | 0.1 | 0.1 |
| Pentacyclic cycloparaffin | 0.0 | 0.0 | 0.0 | 0.1 | 0.2 |
| Hexacyclic cycloparaffin | 0.3 | 0.6 | 0.4 | 0.3 | 0.9 |
| Traction coefficient | | | | | |
| 50N, 25°C, 0.5m/s, Slip ratio 3% | 0.017 | 0.016 | 0.014 | 0.018 | 0.022 |

### [Examples 2-3 to 2-6, Comparative Examples 2-4 to 2-9]

In Examples 2-3 and 2-5, and Comparative Examples 2-4, 2-6, and 2-8, the lubricant base oils of Examples 2-1 and 2-2, or Comparative Examples 2-1 to 2-3, respectively, were used as a sample oil. Furthermore, in Examples 2-4, 2-6, and Comparative Examples 2-5, 2-7, and 2-9, lubricant oil compositions were prepared by adding 0.8 mass% of a package additive (breakdown: 60 mass% of antiwear agent, 25 mass% of antioxidant, 10 mass% of rust inhibitor, and 5 mass% of metal deactivating agent) to the respective lubricant base oils of Examples 2-1 and 2-2, or Comparative Examples 2-1 to 2-3, respectively, to be used as a sample oil.

### [Oil Leakage Test]

With respect to the sample oils of Examples 2-3 to 2-6, and Comparative Examples 2-4 to 2-9, an oil leakage test was performed according to the following procedure.

100 ml of the sample oil is charged in a 200 ml autoclave and an NBR packing is used to be assembled with a tightening torque of 250 N·m using a torque wrench. A two-way cock is used at the upper part and, as a sealing material, a teflon (registered trademark) packing is used to be assembled with a tightening torque of 250 N·m using a torque wrench. After assembling, a pressure is increased to 300 kPa with nitrogen gas. The respective sample oils are subjected to the same operation and are set upside down in a low-temperature thermostat bath that is controlled to be -30±1C°. Results are evaluated by oil leakage from the NBR packing after 48 hours, and with leakage is evaluated as presence and without leakage is evaluated as absence.

The obtained results are shown in Tables 5 and 6.

### [Storage Stability Test]

With respect to the sample oils of Examples 2-3 to 2-6, and Comparative Examples 2-4 to 2-9, a storage stability test was performed according to the following procedure.

In a 100 ml screw vial, an oil is charged to two thirds or more thereof, and each of the test tube is put in a refrigerator of 0±1°C, and the appearance is confirmed after 48 hours. Without change in the appearance is evaluated as without change, and generation of condensation is evaluated as condensation.

### [Energy Saving Property Evaluation Test]

With respect to the lubricant oil compositions of Examples 2-4 and 2-6, and Comparative Examples 2-5, 2-7, and 2-9, an energy saving property evaluation test was performed according to the following procedure.

The energy saving property was evaluated by using a compact hydraulic unit. A variable capacity piston pump was used for a pump in the compact hydraulic unit, the oil amount was 15 L, the oil temperature was 80±2°C and 0°C that considers the time of low-temperature starting, and the input power of a motor when the discharge pressure is varied from 0.8 to 2.4 MPa using a commercial hydraulic oil (0W-20, kinematic viscosity at 40°C: 32.8 mm²/s, viscosity index: 125) was measured. Next, the input power of a motor was measured by using each of the lubricant oil compositions of Examples 3, 4 and Comparative Examples 4 to 6 as a sample oil, and the energy saving property was evaluated based on a difference of power consumption from a sample oil of Comparative Example 7.

The obtained results are shown in Tables 5 and 6.

**[Table 5]**

| | | Example 2-3 | Example 2-4 | Example 2-5 | Example 2-6 |
|---|---|---|---|---|---|
| Base oil | Kind | Example 2-1 | Example 2-1 | Example 2-2 | Example 2-2 |
| | Content (mass%) | 100 | Balance | 100 | Balance |
| Package additive (mass%) | | - | 0.8 | - | 0.8 |
| Characteristics of sample oil | | | | | |
| Kinematic viscosity. mm²/s (40°C) | | 30.3 | 30.5 | 28.2 | 28.4 |
| Viscosity index | | 165 | 164 | 162 | 162 |
| SBV viscosity (mPa·s) | | | | | |
| -20°C | | 29,000 | 29,500 | 3,200 | 3,300 |
| -30°C | | 470,000 | 490,000 | 5,300 | 5,500 |
| Oil leakage test (-20°C) Presence or absence of leakage | | Absence | Absence | Absence | Absence |
| Storage stability (0°C) | | Without change | Without change | Without change | without change |
| Energy saving property | | | | | |
| 80°C | | - | +6.5 | - | +4.9 |
| 0°C | | - | +3.5 | - | +3.1 |

**[Table 6]**

| | | Comp. Example 2-4 | Comp. Example 2-5 | Comp. Example 2-6 | Comp. Example 2-7 | Comp. Example 2-8 | Comp. Example 2-9 |
|---|---|---|---|---|---|---|---|
| Base oil | Kind | Comp. Example 2-1 | Comp. Example 2-1 | Comp. Example 2-2 | Comp. Example 2-2 | Comp. Example 2-3 | Comp. Example 2-3 |
| | Content (mass%) | 100 | Balance | 100 | Balance | 100 | Balance |
| Package additive (mass%) | | - | 0.8 | - | 0.8 | - | 0.8 |

| Characteristics of sample oil | | | | | | | |
|---|---|---|---|---|---|---|---|
| Kinematic viscosity. mm²/s (40°C) | | 29.4 | 29.7 | 26.0 | 26.3 | 30.8 | 31.0 |
| Viscosity index | | 167 | 166 | 154 | 152 | 148 | 146 |

| SBV viscosity (mPa·s) | | | | | | | |
|---|---|---|---|---|---|---|---|
| -20°C | | 122,000 | 123,000 | 2,100 | 2,300 | 1,030 | 1,100 |
| -30°C | | >1,000,000 | >1,000,000 | 4,300 | 4,500 | 1,700 | 1,800 |

| Oil leakage test (-20°C) | | | | | | | |
|---|---|---|---|---|---|---|---|
| Presence or absence of leakage | | Absence | Absence | Presence | Presence | Presence | Presence |
| Storage stability test (0°C) | | Condensation | Condensation | Without change | Without change | Without change | Without change |

| Energy saving property | | | | | | | |
|---|---|---|---|---|---|---|---|
| 80°C | | - | +6.2 | - | +0.6 | - | +0.8 |
| 0°C | | - | -0.3 | - | +1.4 | - | +1.2 |

### [Examples 3-1 to 3-3, Comparative Examples 3-1 to 3-3]

In Examples 3-1 to 3-3 and Comparative Examples 3-1 to 3-3, lubricant base oils shown in Table 7 were each prepared. The lubricant base oils in Examples 3-1 to 3-3 are obtained based on the method for producing a lubricant base oil according to the above-described fourth embodiment. In contrast, the lubricant base oils in Comparative Examples 3-1 to 3-3 are obtained by the conventional method for producing a lubricant base oil. Various characteristics of the respective base oils, and the traction coefficients measured under conditions of a load of 50 N (average hertz pressure 0.60 GPa), a sample oil temperature of 50°C, a circumferential velocity of 1 m/s, and a slip ratio of 3%, and using a 27.4 mm steel ball and a steel disc are shown in Table 7.

**[Table 7]**

| | Example 3-1 | Example 3-2 | Example 3-3 | Comp. Example 3-1 | Comp. Example 3-2 | Comp. Example 3-3 |
|---|---|---|---|---|---|---|
| General physical properties | | | | | | |
| Density, g/cm³ | 0.8054 | 0.8055 | 0.8056 | 0.8057 | 0.8058 | - |
| Flash point, °C | 204 | 202 | 200 | 205 | 197 | - |
| Kinematic viscosity, mm²/s (40°C) | 9.23 | 8.10 | 9.16 | 9.19 | 9.22 | 8.48 |
| (100°C) | 2.70 | 2.45 | 2.66 | 2.70 | 2.65 | 2.51 |
| Viscosity index | 138 | 133 | 131 | 140 | 129 | 127 |
| Pour point, °C | -11 | -22.5 | -27.5 | -7.5 | -30 | -40 |
| Freezing point, °C | -15 | -24 | -28 | -8 | -31 | -43 |
| NOACK, mass% (250°C) | 44.8 | 46.2 | 48.6 | 52.8 | 56.2 | 55.1 |
| Sulfur content, mass ppm | <10 | <10 | <10 | <10 | <10 | <10 |
| Iodine value | 0.08 | 0.07 | 0.08 | 0.07 | 0.09 | 0.07 |
| Aniline point, °C | 111.1 | 110.6 | 110.7 | 112.5 | 111.8 | 112.0 |
| Chromatography analysis | | | | | | |
| Saturated content, mass% | 99.6 | 99.4 | 99.5 | 99.6 | 99.6 | 99.3 |
| Resin content, mass% | 0.3 | 0.3 | 0.3 | 0.2 | 0.2 | 0.3 |
| Aromatic content, mass% | 0.1 | 0.3 | 0.2 | 0.2 | 0.2 | 0.4 |
| Recovery rate, mass% | 100 | 100 | 100 | 100 | 100 | 100 |
| Urea adduct amount, mass% | 9.68 | 4.25 | 4.02 | 12.5 | 0.58 | 0.11 |
| nP, mass% | 15.2 | 23.9 | 22.2 | 14.8 | 32.8 | 37.5 |
| nP Base oil conversion amount, mass% | 1.47 | 1.02 | 0.89 | 1.85 | 0.19 | 0.04 |

| Low-temperature characteristics | | | | | | |
|---|---|---|---|---|---|---|
| SBV viscosity, mP·s (-20°C) | 1,500 | 100 | 110 | 4,500 | 130 | <1000 |
| (-25°C) | 3,100 | 430 | 240 | 37,000 | 200 | - |
| (-30°C) | 19,200 | 2,120 | 1,050 | 49,000 | 780 | 270 |
| (-35°C) | 290,000 | 13,300 | 3,300 | 900,000 | 1,970 | 1,040 |
| (-40°C) | 720,000 | 29,000 | 5,300 | > 1,000,000 | 3,830 | 2,110 |

| ¹³C-NMR | | | | | | |
|---|---|---|---|---|---|---|
| CH | 7.6 | 7.8 | 7.7 | 7.4 | 7.7 | 7.6 |
| CH2 | 76.4 | 76.1 | 75.9 | 76.6 | 76.0 | 75.6 |
| CH3 | 16.0 | 16.1 | 16.2 | 16.0 | 16.3 | 16.8 |
| CH2 main chain | 16.9 | 16.4 | 15.1 | 17.1 | 13.3 | 10.1 |

| EI-MS | | | | | | |
|---|---|---|---|---|---|---|
| Paraffins | 98.2 | 98.1 | 97.9 | 98.3 | 98.0 | 97.7 |
| Monocyclic cycloparaffin | 0.0 | 0.0 | 0.0 | 0.0 | 0.0 | 0.0 |
| Bicyclic cycloparaffin | 1.3 | 1.5 | 1.4 | 1.5 | 1.7 | 1.7 |
| Tricyclic cycloparaffin | 0.3 | 0.4 | 0.3 | 0.1 | 0.3 | 0.3 |
| Tetracyclic cycloparaffin | 0.1 | 0.0 | 0.2 | 0.0 | 0.0 | 0.0 |
| Pentacyclic cycloparaffin | 0.0 | 0.0 | 0.0 | 0.1 | 0.0 | 0.0 |
| Hexacyclic cycloparaffin | 0.1 | 0.0 | 0.2 | 0.0 | 0.0 | 0.3 |
| Alkylbenzenes | 0.0 | 0.0 | 0.0 | 0.0 | 0.0 | 0.0 |

| FD-MS | | | | | | |
|---|---|---|---|---|---|---|
| Paraffins | 79.9 | 76.2 | 70.4 | 82.1 | 68.5 | 67.9 |
| Monocyclic cycloparaffin | 18.5 | 20.1 | 25.8 | 16.3 | 26.4 | 27.3 |
| Bicyclic cycloparaffin | 1.2 | 2.9 | 3.0 | 1.1 | 4.0 | 4.1 |
| Tricyclic cycloparaffin | 0.2 | 0.3 | 0.5 | 0.3 | 0.5 | 0.4 |
| Tetracyclic cycloparaffin | 0.0 | 0.0 | 0.0 | 0.0 | 0.0 | 0.0 |
| Pentacyclic cycloparaffin | 0.1 | 0.0 | 0.1 | 0.0 | 0.1 | 0.0 |
| Hexacyclic cycloparaffin | 0.1 | 0.5 | 0.2 | 0.2 | 0.5 | 0.3 |
| Traction coefficient | 0.013 | 0.014 | 0.015 | 0.011 | 0.016 | 0.019 |

### [Examples 3-4 to 3-6, Comparative Examples 3-4 to 3-6]

In Examples 3-4 to 3-6 and Comparative Examples 3-4 to 3-6, lubricant oil compositions were prepared by adding 8% by mass of a package additive (breakdown: antiwear agent: 12% by mass, ashless dispersant: 50% by mass, pour-point depressant: 1% by mass, antioxidant: 12% by mass, metal-based detergent: 25% by mass) and 5% by mass of a viscosity index improver (polymethacrylate-based, Mw 350,000, effective concentration 50% by mass) to the lubricant base oils of Examples 3-4 to 3-6 and Comparative Examples 3-4 to 3-6, respectively.

### [Oil Leakage Test]

With respect to the sample oils of Examples 3-4 to 3-9, and Comparative Examples 3-4 to 3-9, an oil leakage test was performed according to the following procedure.

More specifically, as a low-temperature leakage test, an actual transmission was used, the sample oil was encapsulated in the transmission to be stored at low temperature, and oil leakage (bleed) was evaluated. The obtained results are shown in Tables 8 and 9.

### [Storage Stability Test]

With respect to the sample oils of Examples 3-4 to 3-9, and Comparative Examples 3-4 to 3-9, a storage stability test was performed according to the following procedure.

In a 100 ml screw vial, an oil is charged to two thirds or more thereof, and each of the test tube is put in a refrigerator of 0±1°C, and the appearance is confirmed after 48 hours. Without change in the appearance is evaluated as without change, and generation of condensation is evaluated as condensation.

### [Low-Temperature Roller Bearing Test]

With respect to the lubricant oils of Examples 3-4, 3-6, and 3-8, and Comparative Examples 3-4, 3-6, and 3-8, a low-temperature roller bearing test was performed using a high-pressure friction tester. More specifically, a measurement site is cooled to 0°C by a cooling jacket under the ordinary pressure condition and the temperature is kept for 4 hours. A cylindrical roller bearing was used as a test piece, and a friction coefficient was evaluated. The obtained results are shown in Tables 8 and 9. The smaller friction coefficient in Table 7 means an excellent reduction in the friction coefficient at the beginning of rolling, in particular, and has a correlation with cold startability by a real machine.

**[Table 8]**

| | | Example 3-4 | Example 3-5 | Example 3-6 | Example 3-7 | Example 3-8 | Example 3-9 |
|---|---|---|---|---|---|---|---|
| Base oil | Kind | Example 3-1 | Example 3-1 | Example 3-2 | Example 3-2 | Example 3-3 | Example 3-3 |
| | Content (mass%) | 100 | Balance | 100 | Balance | Balance | Balance |
| Package additive (mass%) | | - | 8 | - | 8 | - | 8 |
| Viscosity index improver (mass%) | | - | 5 | - | 5 | - | 5 |
| SBV viscosity mPa·s | | | | | | | |
| -40°C | | 720,000 | 320,000 | 29,000 | 16,000 | 5,300 | 5,500 |
| Oil leakage test (-30°C) Presence or absence of leakage | | Absence | Absence | Absence | Absence | Absence | Absence |
| Low-temperature storage stability | | Without change | Without change | Without change | Without change | Without change | Without change |
| Low-temperature roller bearing test Friction coefficient | | 0.020 | - | 0.021 | - | 0.022 | - |

**[Table 9]**

| | | Comp. Example 3-4 | Comp. Example 3-5 | Comp. Example 3-6 | Comp. Example 3-7 | Comp. Example 3-8 | Comp. Example 3-9 |
|---|---|---|---|---|---|---|---|
| Base oil | Kind | Comp. Example 3-1 | Comp. Example 3-1 | Comp. Example 3-2 | Comp. Example 3-2 | Comp. Example 3-3 | Comp. Example 3-3 |
| | Content (mass%) | 100 | Balance | 100 | Balance | Balance | Balance |
| Package additive (mass%) | | - | 8 | - | 8 | - | 8 |
| Viscosity index improver (mass%) | | - | 5 | - | 5 | - | 5 |
| SBV viscosity mPa·s | | | | | | | |
| -40°C | | >1,000,000 | 560,000 | 3,830 | 4,200 | 2,110 | 1,980 |
| Oil leakage test (-30°C) Presence or absence of leakage | | Absence | Absence | Presence | Presence | Presence | Presence |
| Low-temperature storage stability | | Condensation | Condensation | Without change | Without change | Without change | Without change |
| Low-temperature roller bearing test friction coefficient | | 0.052 | - | 0.028 | - | 0.030 | - |

## Claims

1. A lubricant base oil that is a hydrocarbon oil that satisfies any of the following conditions (i), (ii) and (iii):
(i) a hydrocarbon oil having a kinematic viscosity at 100°C of 3.0 to 5.0 mm²/s, a viscosity index of 145 or more, and an SBV viscosity at -20°C of 3,000 to 60,000 mPa·s the SBV viscosity being determined in accordance with ASTM D 5133.
wherein the hydrocarbon oil has a ratio of CH₂ carbons constituting a main chain to all carbons constituting the lubricant base oil of 15% or more in a ¹³C-NMR analysis, wherein ¹³C-NMR analysis is performed under the following conditions:
a diluted sample obtained by adding 3 g of deuterated chloroform to 0.5 g of a sample is used, the measurement temperature is room temperature, the resonant frequency is 100 MHz, and a gated decoupling method is used,
wherein the hydrocarbon oil has a cycloparaffin content of 50% or less in an FD-MS analysis, wherein the FD-MS analysis is performed under the following analysis conditions:
a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min,
(ii) a hydrocarbon oil having a kinematic viscosity at 100°C of 5 to 9 mm²/s, a viscosity index of 155 or more, and an SBV viscosity at -20°C of 3,000 to 30,000 mPa·s,
wherein the hydrocarbon oil has a ratio of CH₂ carbons constituting a main chain to all carbons constituting the lubricant base oil of 20% or more in a ¹³C-NMR analysis, wherein ¹³C-NMR analysis is performed under the following conditions:
a diluted sample obtained by adding 3 g of deuterated chloroform to 0.5 g of a sample is used, the measurement temperature is room temperature, the resonant frequency is 100 MHz, and a gated decoupling method is used,
wherein the hydrocarbon oil has a cycloparaffin content of 60% or less in an FD-MS analysis, wherein the FD-MS analysis is performed under the following analysis conditions:
a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min, and
(iii) a hydrocarbon oil having a kinematic viscosity at 100°C of 2.0 to 3.0 mm²/s, a viscosity index of 130 or more, a pour point of -27.5°C or more, and an SBV viscosity at -30°C of 1,000 to 30,000 mPa·s,
wherein the hydrocarbon oil has a ratio of CH₂ carbons constituting a main chain to all carbons constituting the lubricant base oil of 15% or more in a ¹³C-NMR analysis, wherein ¹³C-NMR analysis is performed under the following conditions:
a diluted sample obtained by adding 3 g of deuterated chloroform to 0.5 g of a sample is used, the measurement temperature is room temperature, the resonant frequency is 100 MHz, and a gated decoupling method is used,
wherein the hydrocarbon oil has a cycloparaffin content of 30% or less in an FD-MS analysis, wherein the FD-MS analysis is performed under the following analysis conditions:
a sample is coated on an emitter, a current is applied to the emitter to heat the coated sample, and a tunneling effect is used in a high electrical field on the emitter surface and in the vicinity of the whisker tip; performing the measurement using JMS-AX505H by JEOL Ltd., an accelerating voltage of 3.0 V and an emitter current of 2 mA/min,
wherein for condition (i), (ii) and (iii) the content of the saturated content in the lubricant base oil on the basis of the total amount of the lubricant base oil is 90% by mass or more; and
wherein for condition (i), (ii) and (iii) the aromatic content in the lubricant base oil on the basis of the total amount of the lubricant base oil is 5% by mass or less.

2. The lubricant base oil according to claim 1, wherein the hydrocarbon oil satisfies the condition (i) and has an SBV viscosity at -30°C of 5,000 to 500,000 mPa·s the SBV viscosity being determined in accordance with ASTM D 5133,

3. The lubricant base oil according to claim 1 or 2, wherein the hydrocarbon oil satisfies the condition (i) and has a freezing point of -20 to -5°C.

4. The lubricant base oil according to claim 1, wherein the hydrocarbon oil satisfies the condition (ii) and has an SBV viscosity at -25°C of 5,000 to 500,000 mPa·s the SBV viscosity being determined in accordance with ASTM D 5133,

5. The lubricant base oil according to claim 1 or 4, wherein the hydrocarbon oil satisfies the condition (ii) and has a freezing point of -15 to -5°C.

6. The lubricant base oil according to claim 1, wherein the hydrocarbon oil satisfies the condition (iii) and has an SBV viscosity at -35°C of 3,000 to 500,000 mPa·s the SBV viscosity being determined in accordance with ASTM D 5133,

7. The lubricant base oil according to claim 1 or 6, wherein the hydrocarbon oil satisfies the condition (iii) and has a freezing point of -30 to -10°C.

## Patentansprüche

1. Schmiermittelbasisöl, welches ein Kohlenwasserstofföl ist, welches beliebige der folgenden Bedingungen (i), (ii) und (iii) erfüllt:
(i) ein Kohlenwasserstofföl mit einer kinematischen Viskosität bei 100 °C von 3,0 bis 5,0 mm²/s, einem Viskositätsindex von 145 oder mehr und einer SBV-Viskosität bei -20 °C von 3.000 bis 60.000 mPa·s, wobei die SBV-Viskosität gemäß ASTM D 5133 bestimmt wird,
wobei das Kohlenwasserstofföl ein Verhältnis von CH₂-Kohlenstoffen, die eine Hauptkette bilden, zu allen Kohlenstoffen, die das Schmiermittelbasisöl bilden, von 15 % oder mehr in einer ¹³C-NMR-Analyse aufweist, wobei die ¹³C-NMR-Analyse unter den folgenden Bedingungen durchgeführt wird:
eine verdünnte Probe, die durch Zugeben von 3 g deuteriertem Chloroform zu 0,5 g einer Probe erhalten wird, wird verwendet, die Messtemperatur ist die Raumtemperatur, die Resonanzfrequenz ist 100 MHz und es wird ein Gated-Decoupling-Verfahren verwendet,
wobei das Kohlenwasserstofföl einen Cycloparaffingehalt von 50 % oder weniger in einer FD-MS-Analyse aufweist, wobei die FD-MS-Analyse unter den folgenden Analysebedingungen durchgeführt wird:
eine Probe wird auf einen Emitter aufgetragen, ein Strom wird an den Emitter angelegt, um die aufgetragene Probe zu erwärmen, und ein Tunneleffekt wird in einem hohen elektrischen Feld an der Emitteroberfläche und in der Nähe der Whisker-Spitze verwendet; wobei die Messung unter Verwendung von JMS-AX505H von JEOL Ltd., einer Beschleunigungsspannung von 3,0 V und einem Emitterstrom von 2 mA/min durchgeführt wird,
(ii) ein Kohlenwasserstofföl mit einer kinematischen Viskosität bei 100 °C von 5 bis 9 mm²/s, einem Viskositätsindex von 155 oder mehr und einer SBV-Viskosität bei -20 °C von 3.000 bis 30.000 mPa·s,
wobei das Kohlenwasserstofföl ein Verhältnis von CH₂-Kohlenstoffen, die eine Hauptkette bilden, zu allen Kohlenstoffen, die das Schmiermittelbasisöl bilden, von 20 % oder mehr in einer ¹³C-NMR-Analyse aufweist, wobei die ¹³C-NMR-Analyse unter den folgenden Bedingungen durchgeführt wird:
eine verdünnte Probe, die durch Zugeben von 3 g deuteriertem Chloroform zu 0,5 g einer Probe erhalten wird, wird verwendet, die Messtemperatur ist die Raumtemperatur, die Resonanzfrequenz ist 100 MHz und es wird ein Gated-Decoupling-Verfahren verwendet,
wobei das Kohlenwasserstofföl einen Cycloparaffingehalt von 60 % oder weniger in einer FD-MS-Analyse aufweist, wobei die FD-MS-Analyse unter den folgenden Analysebedingungen durchgeführt wird:
eine Probe wird auf einen Emitter aufgetragen, ein Strom wird an den Emitter angelegt, um die aufgetragene Probe zu erwärmen, und ein Tunneleffekt wird in einem hohen elektrischen Feld an der Emitteroberfläche und in der Nähe der Whisker-Spitze verwendet; wobei die Messung unter Verwendung von JMS-AX505H von JEOL Ltd., einer Beschleunigungsspannung von 3,0 V und einem Emitterstrom von 2 mA/min durchgeführt wird, und
(iii) ein Kohlenwasserstofföl mit einer kinematischen Viskosität bei 100 °C von 2,0 bis 3,0 mm²/s, einem Viskositätsindex von 130 oder mehr, einem Pourpoint von -27,5 °C oder mehr und einer SBV-Viskosität bei -30 °C von 1.000 bis 30.000 mPa·s,
wobei das Kohlenwasserstofföl ein Verhältnis von CH₂-Kohlenstoffen, die eine Hauptkette bilden, zu allen Kohlenstoffen, die das Schmiermittelbasisöl bilden, von 15 % oder mehr in einer ¹³C-NMR-Analyse aufweist, wobei die ¹³C-NMR-Analyse unter den folgenden Bedingungen durchgeführt wird:
eine verdünnte Probe, die durch Zugeben von 3 g deuteriertem Chloroform zu 0,5 g einer Probe erhalten wird, wird verwendet, die Messtemperatur ist die Raumtemperatur, die Resonanzfrequenz ist 100 MHz und es wird ein Gated-Decoupling-Verfahren verwendet,
wobei das Kohlenwasserstofföl einen Cycloparaffingehalt von 30 % oder weniger in einer FD-MS-Analyse aufweist, wobei die FD-MS-Analyse unter den folgenden Analysebedingungen durchgeführt wird:
eine Probe wird auf einen Emitter aufgetragen, ein Strom wird an den Emitter angelegt, um die aufgetragene Probe zu erwärmen, und ein Tunneleffekt wird in einem hohen elektrischen Feld an der Emitteroberfläche und in der Nähe der Whisker-Spitze verwendet; wobei die Messung unter Verwendung von JMS-AX505H von JEOL Ltd., einer Beschleunigungsspannung von 3,0 V und einem Emitterstrom von 2 mA/min durchgeführt wird,
wobei für Bedingung (i), (ii) und (iii) der Gehalt des gesättigten Gehalts in dem Schmiermittelbasisöl, bezogen auf die Gesamtmenge des Schmiermittelbasisöls, 90 Massen% oder mehr beträgt; und
wobei für die Bedingung (i), (ii) und (iii) der aromatische Gehalt in dem Schmiermittelbasisöl, bezogen auf die Gesamtmenge des Schmiermittelbasisöls, 5 Massen% oder weniger beträgt.

2. Schmiermittelbasisöl gemäß Anspruch 1, wobei das Kohlenwasserstofföl die Bedingung (i) erfüllt und eine SBV-Viskosität bei -30 °C von 5.000 bis 500.000 mPa·s aufweist, wobei die SBV-Viskosität gemäß ASTM D 5133 bestimmt wird.

3. Schmiermittelbasisöl gemäß Anspruch 1 oder 2, wobei das Kohlenwasserstofföl die Bedingung (i) erfüllt und einen Gefrierpunkt von -20 bis -5 °C aufweist.

4. Schmiermittelbasisöl gemäß Anspruch 1, wobei das Kohlenwasserstofföl die Bedingung (ii) erfüllt und eine SBV-Viskosität bei -25 °C von 5.000 bis 500.000 mPa·s aufweist, wobei die SBV-Viskosität gemäß ASTM D 5133 bestimmt wird.

5. Schmiermittelbasisöl gemäß Anspruch 1 oder 4, wobei das Kohlenwasserstofföl die Bedingung (ii) erfüllt und einen Gefrierpunkt von -15 bis -5 °C aufweist.

6. Schmiermittelbasisöl gemäß Anspruch 1, wobei das Kohlenwasserstofföl die Bedingung (iii) erfüllt und eine SBV-Viskosität bei -35 °C von 3.000 bis 500.000 mPa·s aufweist, wobei die SBV-Viskosität gemäß ASTM D 5133 bestimmt wird.

7. Schmiermittelbasisöl gemäß Anspruch 1 oder 6, wobei das Kohlenwasserstofföl die Bedingung (iii) erfüllt und einen Gefrierpunkt von -30 bis -10 °C aufweist.

## Revendications

1. Huile de base pour lubrifiant qui est une huile hydrocarbure qui satisfait n'importe laquelle des conditions suivantes (i), (ii) et (iii) :
(i) une huile hydrocarbure ayant une viscosité cinématique à 100°C de 3,0 à 5,0 mm²/s, un indice de viscosité de 145 ou plus, et une viscosité SBV à -20°C de 3 000 à 60 000 mPa·s la viscosité SBV étant déterminée selon la norme ASTM D 5133,
où l'huile hydrocarbure présente un rapport des carbones CH₂ constituant une chaîne principale à l'ensemble des carbones constituant l'huile de base pour lubrifiant de 15 % ou plus dans une analyse de RMN ¹³C, où l'analyse de RMN ¹³C est effectuée sous les conditions suivantes :
un échantillon dilué obtenu par l'addition de 3 g de chloroforme deutérié à 0,5 g d'un échantillon est utilisé, la température de mesure est la température ambiante, la fréquence de résonance est 100 MHz, et un procédé de découplage à déclenchement périodique est utilisé,
où l'huile hydrocarbure présente une teneur en cycloparaffine de 50 % ou moins dans une analyse FD-MS, où l'analyse FD-MS est effectuée sous les conditions d'analyse suivantes :
un échantillon est revêtu sur un émetteur, un courant est appliqué à l'émetteur pour chauffer l'échantillon revêtu, et un effet tunnel est utilisé dans un champ électrique élevé sur la surface de l'émetteur et à proximité de la pointe de trichite, la réalisation de la mesure en utilisant la norme JMS-AX505H par JEOL Ltd., une tension d'accélération de 3,0 V et un courant d'émission de 2 mA/min,
(ii) une huile hydrocarbure ayant une viscosité cinématique à 100°C de 5 à 9 mm²/s, un indice de viscosité de 155 ou plus, et une viscosité SBV à -20°C de 3 000 à 30 000 mPa·s,
où l'huile hydrocarbure présente un rapport des carbones CH₂ constituant une chaîne principale à l'ensemble des carbones constituant l'huile de base pour lubrifiant de 20 % ou plus dans une analyse de RMN ¹³C, où l'analyse de RMN ¹³C est effectuée sous les conditions suivantes :
un échantillon dilué obtenu par l'addition de 3 g de chloroforme deutérié à 0,5 g d'un échantillon est utilisé, la température de mesure est la température ambiante, la fréquence de résonance est 100 MHz, et un procédé de découplage à déclenchement périodique est utilisé,
où l'huile hydrocarbure présente une teneur en cycloparaffine de 60 % ou moins dans une analyse FD-MS, où l'analyse FD-MS est effectuée sous les conditions d'analyse suivantes :
un échantillon est revêtu sur un émetteur, un courant est appliqué à l'émetteur pour chauffer l'échantillon revêtu, et un effet tunnel est utilisé dans un champ électrique élevé sur la surface de l'émetteur et à proximité de la pointe de trichite ; la réalisation de la mesure en utilisant la norme JMS-AX505H par JEOL Ltd., une tension d'accélération de 3,0 V et un courant d'émission de 2 mA/min, et
(iii) une huile hydrocarbure ayant une viscosité cinématique à 100°C de 2,0 à 3,0 mm²/s, un indice de viscosité de 130 ou plus, un point d'écoulement de -27,5°C ou plus, et une viscosité SBV à -30°C de 1 000 à 30 000 mPa·s,
où l'huile hydrocarbure présente un rapport des carbones CH₂ constituant une chaîne principale à l'ensemble des carbones constituant l'huile de base pour lubrifiant de 15 % ou plus dans une analyse de RMN ¹³C, où l'analyse de RMN ¹³C est effectuée sous les conditions suivantes :
un échantillon dilué obtenu par l'addition de 3 g de chloroforme deutérié à 0,5 g d'un échantillon est utilisé, la température de mesure est la température ambiante, la fréquence de résonance est 100 MHz, et un procédé de découplage à déclenchement périodique est utilisé,
où l'huile hydrocarbure présente une teneur en cycloparaffine de 30 % ou moins dans une analyse FD-MS, où l'analyse FD-MS est effectuée sous les conditions d'analyse suivantes :
un échantillon est revêtu sur un émetteur, un courant est appliqué à l'émetteur pour chauffer l'échantillon revêtu, et un effet tunnel est utilisé dans un champ électrique élevé sur la surface de l'émetteur et à proximité de la pointe de trichite ; la réalisation de la mesure en utilisant la norme JMS-AX505H par JEOL Ltd., une tension d'accélération de 3,0 V et un courant d'émission de 2 mA/min,
où pour la condition (i), (ii) et (iii) la teneur saturée dans l'huile de base pour lubrifiant sur la base de la quantité totale de l'huile de base pour lubrifiant est de 90 % en masse ou plus ; et
où pour la condition (i), (ii) et (iii) la teneur en composés aromatiques dans l'huile de base pour lubrifiant sur la base de la quantité totale de l'huile de base pour lubrifiant est de 5 % en masse ou moins.

2. Huile de base pour lubrifiant selon la revendication 1, dans laquelle l'huile hydrocarbure satisfait la condition (i) et présente une viscosité SBV à -30°C de 5 000 à 500 000 mPa·s la viscosité SBV étant déterminée selon la norme ASTM D 5133.

3. Huile de base pour lubrifiant selon la revendication 1 ou 2, dans laquelle l'huile hydrocarbure satisfait la condition (i) et présente un point de congélation de -20 à -5°C.

4. Huile de base pour lubrifiant selon la revendication 1, dans laquelle l'huile hydrocarbure satisfait la condition (ii) et présente une viscosité SBV à -25°C de 5 000 à 500 000 mPa·s la viscosité SBV étant déterminée selon la norme ASTM D 5133.

5. Huile de base pour lubrifiant selon la revendication 1 ou 4, dans laquelle l'huile hydrocarbure satisfait la condition (ii) et présente un point de congélation de -15 à -5°C.

6. Huile de base pour lubrifiant selon la revendication 1, dans laquelle l'huile hydrocarbure satisfait la condition (iii) et présente une viscosité SBV à -35°C de 3 000 à 500 000 mPa·s la viscosité SBV étant déterminée selon la norme ASTM D 5133.

7. Huile de base pour lubrifiant selon la revendication 1 ou 6, dans laquelle l'huile hydrocarbure satisfait la condition (iii) et présente un point de congélation de -30 à -10°C.
